

## 1

3,032,485

## ELECTROLYTIC BATH FOR USE IN ELECTRODEPOSITION OF FERROMAGNETIC COMPOSITIONS

Ignatius Tsu, Jerome S. Sallo, and Robert D. Fisher, Dayton, Ohio, and Harsukh J. Modi, West Lafayette, Ind., assignors to The National Cash Register Company, Dayton, Ohio, a corporation of Maryland  
 No Drawing. Filed Oct. 1, 1958, Ser. No. 764,522  
 25 Claims. (Cl. 204—43)

This invention relates generally to the manufacture of ferromagnetic memory elements such as wires, bobbin and toroidal shaped cores, and the like, for use in present day electronic computers and data processors, and more specifically relates to new and improved electrolytic baths for use in the manufacturing of such elements which possess greatly improved magnetic characteristics than heretofore possible.

In most electronic computer and data processor applications, it is generally highly desirable that the magnetic memory elements be relatively small in size, require negligible expenditure of time and effort in order to be electrically connected in circuit, be physically sturdy and economical to manufacture utilizing mass production techniques, possess relatively high magnetic remanence and relatively low magnetic coercivity properties, be readily adaptable to fast switching operations measured in fractions of microseconds, and additionally, possess substantially rectangular hysteresis characteristics resulting in substantially high signal-to-noise ratios.

Various attempts have heretofore been made to produce such magnetic memory elements for information storage purposes by electroplating an electrically conductive carrier with a relatively thin coating of an alloy having magnetic properties. Even though present day electroplating techniques possess practically unlimited potentialities in the manufacture of such elements, to date however, to the knowledge of applicants there is yet to be produced thereby any memory element which possesses all of the above-mentioned characteristics.

Consequently, the primary object of the present invention is to devise a new and improved aqueous electrolytic bath for utilization in the process of electrodeposition of a ferromagnetic coating onto an electrically conductive carrier whereby magnetic memory elements are produced which possess all of the above-mentioned characteristics.

Briefly, in accordance with the present invention, such a bath includes as essential constituents iron ions in a concentration in the range of .7 to 16 grams per liter, 50 nickel ions in a concentration in the range of 3 to 10 grams per liter, molybdenum (VI) in a concentration in the range of .1 to 1 gram per liter, and a complexing agent.

More specifically, the plating bath preferably contains simple salts of iron, nickel, and molybdenum in complexed form wherein iron is initially added as either a ferrous salt such as ferrous chloride ( $FeCl_2 \cdot 4H_2O$ ) or as a ferric salt such as ferric chloride ( $FeCl_3 \cdot 6H_2O$ ). From the standpoint of economic availability, the chlorides of iron are preferred, however, any salt of iron may be used provided the anion does not cause precipitation in the overall system.

Nickel is preferably added to the plating bath as a simple nickel chloride salt ( $NiCl_2 \cdot 6H_2O$ ). However, following the addition, several nickel species may appear as free nickel ions, nickel amine complexes, nickel chel-

## 2

ates, nickel addition agent complexes, and nickel complexes with other added metal salts. Nickel may be added in the form of other salts, as an illustrative example nickel sulfate ( $NiSO_4 \cdot 6H_2O$ ) provided precipitation does not occur. The form in which nickel exists in a given system depends upon many factors such as the nickel concentration, pH, ammonium ion concentration, chelating agent concentration, iron concentration, addition agent concentration, complexing agent concentration, 10 temperature, and concentration of other metal salts. It is by varying these factors that a wide range of magnetic properties is obtained. In addition, the nickel species in the bulk of the solution are not necessarily the same as the nickel species occurring in the so-called "double layer" at the cathode. It is the latter species from which deposition actually occurs and which is of major importance in determining the magnetic properties of the deposit.

Molybdenum (VI) has an appreciable effect in the plating bath and it is preferably added to the bath in the form of sodium molybdate ( $Na_2MoO_4 \cdot 2H_2O$ ). However, molybdenum may be added in the form of other compounds provided they cause no precipitation in the overall system. For example, molybdenum may be added in 25 the form of molybdic acid ( $H_2MoO_4$ ), phosphomolybdic acid ( $P_2O_5 \cdot 24MoO_3 \cdot XH_2O$ ), potassium molybdate ( $K_2MoO_4 \cdot 2H_2O$ )

ammonium molybdate [ $(NH_4)_2MoO_4 \cdot 2H_2O$ ], ammonium 30 heptamolybdate [ $(NH_4)_6Mo_7O_{24} \cdot 4H_2O$ ], molybdenum trioxide ( $MoO_3$ ), etc. However, the concentration of molybdenum (VI) is critical and the optimum concentration depends upon the overall condition of the system. In fact, in the preferred bath if the molybdate concentration 35 is excessive, for example an ionic concentration thereof in excess of approximately 2 grams per liter, little or no deposit results. Molybdate in such bath has been found to effect the plating bath similarly to addition agents in that, for example, molybdate lowers the discharge potential of the plating process and is believed to 40 complex with the iron and/or nickel constituents in the bath.

Due to the fact that even the hydroxides of iron begin to precipitate even in acid solutions, it is desirable to utilize a complexing agent to maintain the plating bath in solution. The preferred complexing agent for this purpose is ammonium citrate [ $(NH_4)_2HC_6H_5O_7$ ]. However, any material which forms a complex with the iron ions of sufficient solubility and stability is a suitable complexing agent. For example, complexing agents which may be used with equal success are sodium citrate



and potassium citrate ( $K_3C_6H_5O_7 \cdot 2H_2O$ ). Various acids such as citric acid ( $H_3C_6H_5O_7 \cdot XH_2O$ ), glycolic acid ( $C_2H_4O_3 \cdot XH_2O$ ), aspartic acid ( $C_4H_7O_4N \cdot XH_2O$ ), and the sodium salt of ethylenediaminetetraacetic acid



etc. may be used, provided there is no breakdown of the complex for example anodic oxidation during the plating process which might form oxidation products at the anode thus modifying the plating bath and, consequently, modifying the magnetic properties of the cathode deposit.

In the present invention, it is believed that the essential function of the complexing agent is to provide a

soluble reservoir of iron, nickel, and/or molybdenum (VI) ions from which are formed, through dynamic equilibria, the species from which the deposition actually occurs. The complexing agent must be of a concentration in the bath to supply the iron, nickel and molybdenum (VI) species rapidly enough through equilibria to provide a suitable concentration of species for deposition, and yet, not rapidly enough to form an appreciable amount of other species whose solubility limits are exceeded to cause precipitation in the bath. Since the complexing agent partially determines the concentration of the reactive species present in the plating bath, the choice of the particular complexing agent has an effect on the composition and structure, and consequently the magnetic properties of the cathode deposit, which influence may be modified by the other constituents of the plating system. In the preferred ferrous plating bath, it is desirable that a minimum molar ratio of 1 to 1 be maintained between the relative citrate and ferrous ion concentrations.

Ammonia is preferably added to the plating bath in the form of ammonium hydroxide ( $\text{NH}_4\text{OH}$ ) to control the pH thereof. Even though it is possible to utilize the plating baths, in accordance with the present invention, to prepare cathode deposits having magnetic properties without the addition of ammonia, it is desirable that the baths have a pH within the range of 7.5 to 9.5, preferably 8.5. Ammonia, aside from controlling the pH, is believed to modify the bath through complex formations and to be part of the reservoir complexes from which deposition occurs. Amines have been found to be less suitable than ammonia for controlling the bath pH, however, non-complexing bases such as sodium hydroxide ( $\text{NaOH}$ ) and potassium hydroxide ( $\text{KOH}$ ) may be used with equal success, provided the amounts added to the citrate baths are of insufficient quantity to cause precipitation therein. As the plating bath is operated within a temperature range of 80° C. to 95° C., preferably 90° C., the ammonia concentration is depleted due to evaporation and, consequently, it is necessary to continuously replenish the bath with ammonium hydroxide to maintain the pH thereof at the preferred 8.5 value.

Ammonium is preferably added to the plating bath in the form of ammonium chloride ( $\text{NH}_4\text{Cl}$ ). As the ammonium ions exert a common ion effect on the ammonia complexes, they are believed to influence the concentration of the ionic species present in the system and thereby effect the structure and magnetic properties of the electrodeposit. Other ammonium salts i.e. ammonium sulfate [ $(\text{NH}_4)_2\text{SO}_4$ ], may be used with equal success provided precipitation does not occur in the bath as a result of the addition.

Shown below in charts I and II, are two forms of new and improved aqueous electrolytic baths having preferred constituent concentrations in accordance with the teachings of the present invention, for use in the process of deposition of an iron-nickel-molybdenum coating on an electrically conductive carrier, in which process the carrier is subjected as a cathode to electrolytic action in the bath, during which the coating formed thereon possesses greatly improved magnetic characteristics. It is to be noted that in the upper half of each chart, is given the concentration of each compound in the actual bath measured in grams per liter of aqueous solution; in the lower half of each chart, is the concentration given in grams per liter of aqueous solution of each constituent present in solution as contributed by each compound. In each instance, the minimum, optimum, and maximum concentrations for each constituent is given in tabular form. It is to be understood of course that the upper and lower concentration limits of each compound and constituent of the bath are not critical in that they specifically define limits above and below which is a definite zone of demarcation of all useful magnetic properties possessed by the cathode deposit.

| Plating Bath Compounds                                                         | Minim-<br>um | Opti-<br>mum | Maxi-<br>mum |
|--------------------------------------------------------------------------------|--------------|--------------|--------------|
| Ferrous Chloride ( $\text{FeCl}_2 \cdot 4\text{H}_2\text{O}$ )                 | 45           | 50           | 55           |
| Nickel Chloride ( $\text{NiCl}_2 \cdot 6\text{H}_2\text{O}$ )                  | 10           | 20           | 40           |
| Sodium Molybdate ( $\text{Na}_2\text{MoO}_4 \cdot 2\text{H}_2\text{O}$ )       | .5           | 1            | 3            |
| Ammonium Citrate [ $(\text{NH}_4)_2\text{H}_2\text{C}_6\text{H}_5\text{O}_7$ ] | 105          | 125          | 135          |
| Ammonium Chloride ( $\text{NH}_4\text{Cl}$ )                                   | 35           | 50           | 100          |

5

| Plating Bath Constituents     | Minim-<br>um | Opti-<br>mum | Maxi-<br>mum |
|-------------------------------|--------------|--------------|--------------|
| Ferrous Ion Concentration     | 12           | 14           | 16           |
| Nickel Ion Concentration      | 3            | 5            | 10           |
| Molybdenum (VI) Concentration | .1           | .4           | 1            |
| Citrate Ion Concentration     | 88           | 104          | 113          |
| Ammonium Ion Concentration    | 12           | 17           | 34           |

10

| Plating Bath Compounds                                                         | Minim-<br>um | Opti-<br>mum | Maxi-<br>mum |
|--------------------------------------------------------------------------------|--------------|--------------|--------------|
| Ferric Chloride ( $\text{FeCl}_3 \cdot 6\text{H}_2\text{O}$ )                  | 4            | 6            | 15           |
| Nickel Chloride ( $\text{NiCl}_2 \cdot 6\text{H}_2\text{O}$ )                  | 10           | 20           | 40           |
| Sodium Molybdate ( $\text{Na}_2\text{MoO}_4 \cdot 2\text{H}_2\text{O}$ )       | .5           | 1            | 3            |
| Ammonium Citrate [ $(\text{NH}_4)_2\text{H}_2\text{C}_6\text{H}_5\text{O}_7$ ] | 40           | 50           | 125          |
| Ammonium Chloride ( $\text{NH}_4\text{Cl}$ )                                   | 25           | 50           | 75           |

15

| Plating Bath Constituents     | Minim-<br>um | Opti-<br>mum | Maxi-<br>mum |
|-------------------------------|--------------|--------------|--------------|
| Ferric Ion Concentration      | .7           | 1            | 3            |
| Nickel Ion Concentration      | 3            | 5            | 10           |
| Molybdenum (VI) Concentration | .1           | .4           | 1            |
| Citrate Ion Concentration     | 33           | 42           | 104          |
| Ammonium Ion Concentration    | 8            | 17           | 25           |

20

| Plating Bath Compounds                                                         | Minim-<br>um | Opti-<br>mum | Maxi-<br>mum |
|--------------------------------------------------------------------------------|--------------|--------------|--------------|
| Ferric Chloride ( $\text{FeCl}_3 \cdot 6\text{H}_2\text{O}$ )                  | 4            | 6            | 15           |
| Nickel Chloride ( $\text{NiCl}_2 \cdot 6\text{H}_2\text{O}$ )                  | 10           | 20           | 40           |
| Sodium Molybdate ( $\text{Na}_2\text{MoO}_4 \cdot 2\text{H}_2\text{O}$ )       | .5           | 1            | 3            |
| Ammonium Citrate [ $(\text{NH}_4)_2\text{H}_2\text{C}_6\text{H}_5\text{O}_7$ ] | 40           | 50           | 125          |
| Ammonium Chloride ( $\text{NH}_4\text{Cl}$ )                                   | 25           | 50           | 75           |

25

| Plating Bath Constituents     | Minim-<br>um | Opti-<br>mum | Maxi-<br>mum |
|-------------------------------|--------------|--------------|--------------|
| Ferric Ion Concentration      | .7           | 1            | 3            |
| Nickel Ion Concentration      | 3            | 5            | 10           |
| Molybdenum (VI) Concentration | .1           | .4           | 1            |
| Citrate Ion Concentration     | 33           | 42           | 104          |
| Ammonium Ion Concentration    | 8            | 17           | 25           |

30

Even though the new and improved aqueous electrolytic baths, just described, find utility in any of the numerous present day electroplating process, a preferred process will be described utilizing the baths of the present invention whereby magnetic data storage devices of the "twistor" type, such as that shown and described in pending application Serial No. 696,987, by J. R. Anderson, et al., filed November 18, 1957, and assigned to the present assignee, are fabricated and exhibit improved magnetic characteristics than heretofore possible.

After the electrolytic bath has been prepared, either I or II, and the pH adjusted to a value in the range of 7.5 to 9.5, preferably 8.5, the temperature is then adjusted to a value in the range of 80° C. to 95° C., preferably 90° C., even though the bath may successfully be operated at ordinary room temperature. The bath is then introduced into a conventional rubber-lined steel plating tank, or an equivalent inert container. The carrier, onto which the deposit is to be formed, may be of any of a variety of non-magnetic electrically conductive materials such as alloys of copper, aluminum, brass, bronze, etc. In fact the carrier may even be of such materials as glass, plastic, or ceramic, assuming of course that it has previously been provided with a suitable electrically conductive skin covering in a well-known manner. However, in the fabrication of the "twistor" types of bistable magnetic data storage devices, as disclosed in the aforementioned copending application, it is preferred that the carrier be a Phosphor-bronze wire having a diameter of approximately 9 mils. It is, of course, necessary that the metallic carrier be cleaned before plating through the use of the conventional alkaline-acid-water methods which are well known in the plating industry.

35

In the "twistor" type of device it is desirable to secure a relatively thin deposit on the carrier in the order of one ten-thousandth of an inch so as to maintain eddy current losses therein at a minimum during operation of the device, and yet be thick enough to insure adequate output and not fracture when torsional stresses are applied

70

75

thereto as described in the copending application. Consequently, it is desirable that the carrier be exposed as a cathode in the bath for only a short period of time, i.e. from approximately 30 seconds to 3 minutes, preferably in the order of 2 minutes depending upon, of course, the cathode current density to be used in the plating process. To accomplish this, the process is made a continuous one whereby the carrier is moved through the bath at a constant speed, by any well known means, with electrical contact at all times maintained with the carrier to supply current thereto. The carrier is preferably centrally encompassed at all times while in the bath by a helical-shaped anode having a coil diameter of approximately one inch and composed of an electrically conductive wire of approximately 50 mils in diameter.

The choice of anode material may not arbitrarily be made, however, iron-nickel, and iron-nickel-molybdenum may successfully be used provided the anode is "bagged" in a conventional manner to prevent sludge formations at the anode from entering the bath solution. One of the important factors associated with the choice of anode material is oxidation in the system. When using bath I, ferrous ions are converted to ferric ions due to oxidation of the bath and high concentration of ferric ions therein is to be avoided. Inert anodes such as platinum, or the like, may be used provided they do not lead to excessive oxidation of the system. It has been found that in each of baths I and II, molybdenum anodes are preferred as they do not have to be "bagged" and tend to replenish the bath with molybdenum. However, even when a molybdenum anode is used, it is necessary to continually add molybdate solution to the bath in order to maintain the molybdate concentration constant at the desired value. Additionally, it is necessary that nickel and iron solutions be continually added to the bath to also maintain the concentrations thereof constant at their respective values during the plating process.

The current density involved in the deposition process is not critical and may range, for example, from 150 to 500, preferably 250, amperes per square foot of carrier surface area exposed in bath I and from 200 to 1000, preferably 250, amperes per square foot of carrier surface area exposed in bath II. The current density primarily determines the rate of deposition of the metallic ions onto the cathode. This affects the rate of diffusion into the cathode film which influences the amount of depositing species which must be in equilibrium with the reservoir complexes. Consequently, the bath and current density must be compatible and the current density cannot arbitrarily be chosen. For example, any addition agents in the system are less effective at relatively high current densities and, consequently, larger quantities must be used. As the current density is one of the prime factors which determine the structure of the deposit, it is generally necessary to modify the plating system to permit the use of a specific current density.

On emergence from the plating bath, the ferromagnetic element is rinsed and dried and is then ready to be operated as a coincident current "twistor" type of data storage device in the following manner as fully described in the aforementioned copending application:

The core, along with the ferromagnetic coating, is simultaneously stretched and twisted and the ends thereof are thereafter held in a fixed position. As a result of the stretching and twisting, the easy direction of magnetization of the coating is oriented from a direction substantially parallel to the longitudinal axis of the core to one of substantially helical configuration about the body of the core and throughout its length as the threads of a screw. Such a ferromagnetic coating has been found to possess a substantially high positive and negative magnetic remanence and substantially rectangular hysteresis characteristic. Consequently, selected length portions of the coating, in the direction of twist, are allowed to attain one or other of the two stable states, namely, a residual

positive or negative remanent induction. A magnetic field along the direction of twist of  $\pm H$  oersteds switches the length portions from one state to another, whereas a field of  $\pm H/2$  oersteds produces only negligible changes in the remanent induction. A plurality of similar coils, of say 20 turns each, are separately wound about the coated wire and are positioned in a spaced side-by-side relationship with respect to one another to define a corresponding plurality of helical-path length portions of ferromagnetic material. Storage of binary information in a select length portion of coating is accomplished by sending a current impulse equal in magnitude to  $(I_1)$  into the conductive wire of the common core and simultaneously sending a current impulse equal in magnitude to  $(I_2)$  into the select coil in such directions that the vector summation of the magnetic field produced by the two coincident currents are equal in magnitude to  $\pm H$  oersteds and is oriented in the same direction as the twist or easy direction of magnetization of the coating.

During reading of the selected length portion of the coating, the core is preferably pulsed to individually develop a magnetic field of  $\pm H$  oersteds in the opposite direction from the magnetic field developed during storage of the function. In response to the read impulse, an electrical signal is or is not available between the ends of the corresponding coil according to whether the binary information 1 or 0, respectively, has been established in the particular length section of the coating as represented by its remanent state.

Listed below in chart form are the electrical operational characteristics of two "twistor" data storage elements fabricated by the previously described plating process which utilize each of the unique ferrous and ferric baths previously described and differ only in wire size of carrier.

|    |                                                                                | Ferrous Bath                 | Ferric Bath              |
|----|--------------------------------------------------------------------------------|------------------------------|--------------------------|
| 40 | Degrees of twist/inch of storage element length                                | 145.....                     | 10.                      |
|    | Approx. one-half coincident current in core for storage of binary data.....ma. | 200 ma.....                  | 75 ma.                   |
|    | Approx. one-half coincident current in coil for storage of binary data.....ma. | 100 ma.....                  | 50 ma.                   |
|    | Full coincident current in coil for reading of stored binary data.....ma.      | 500 ma.....                  | 500 ma.                  |
|    | Voltage output across ends of core during reading of binary 1 data.....mv.     | 70 mv.....                   | 75 mv.                   |
| 45 | Signal to noise ratio.....                                                     | 5.....                       | 75.                      |
|    | Minimum switching time..... $\mu$ sec.                                         | Less than 0.3 micro sec..... | Less than 0.3 micro sec. |
|    | Diameter of carrier.....mils.                                                  | Approx. 9 mils.              | Approx. 9 mils.          |

|    |                                                                                | Ferrous Bath | Ferric Bath |
|----|--------------------------------------------------------------------------------|--------------|-------------|
| 55 | Degrees of twist/inch of storage element length                                | 360.....     | 10          |
|    | Approx. one-half coincident current in core for storage of binary data.....ma. | 85.....      | 60          |
|    | Approx. one-half coincident current in coil for storage of binary data.....ma. | 55.....      | 40          |
|    | Full coincident current in coil for reading of stored binary data.....ma.      | 300.....     | 300         |
|    | Voltage output across ends of core during reading of binary 1 data.....mv.     | 70.....      | 75          |
| 60 | Signal to noise ratio..... $\mu$ sec.                                          | 5.....       | 75          |
|    | Minimum switching time..... $\mu$ sec.                                         | < 3          | < 3         |
|    | Diameter of carrier.....mils.                                                  | 3            | 3           |

In each of the storage elements, the coercivity is less than 2 oersteds and the squareness of the hysteresis loop approximately .99. Consequently, it can thus be seen that by the use of the unique aqueous electrolytic baths, in accordance with the present invention, new and improved ferromagnetic data storage elements are fabricated by electroplating a ferromagnetic coating onto an electrically conductive carrier. Such elements, in addition to possessing greatly improved magnetic characteristics than heretofore possible, are readily adaptable to be fabricated by mass production techniques thereby maintaining the cost thereof at a minimum, and are ideally suited for

incorporation in present day electronic data processors and computers.

While particular embodiments of the invention have been shown and described, it will be obvious to those skilled in the art of electrodeposition of ferromagnetic materials, that changes and modifications may be made without departing from the invention in its broader aspects, and therefore, the aim in the appended claims is to cover all such changes and modifications as fall within the true spirit and scope of the invention.

What is claimed is:

1. An aqueous electrolytic bath for use in the process of deposition of a ferromagnetic coating on an electrically conductive carrier in which process said carrier is subjected as a cathode to electrolytic action in said bath, said bath having a pH in the range of 7.5 to 9.5 and including as essential constituents ferrous ions in a concentration in the range of 12 to 16 grams per liter, nickel ions in a concentration in the range of 3 to 10 grams per liter, molybdenum (VI) in a concentration in the range of .1 to 1 gram per liter, and a complexing agent capable of forming soluble ferrous, nickel, and molybdenum (VI) complexes and being of sufficient concentration to prevent precipitation of ferrous, nickel, and molybdenum (VI) ions.

2. An aqueous electrolytic bath for use in the process of deposition of a ferromagnetic coating on an electrically conductive carrier in which process said carrier is subjected as a cathode to electrolytic action in said bath, said bath having a pH of approximately 8.5 and including as essential constituents ferrous ions in a concentration approximately 14 grams per liter, nickel ions in a concentration approximately 5 grams per liter, molybdenum (VI) in a concentration approximately .4 gram per liter, and a complexing agent capable of forming soluble ferrous, nickel, and molybdenum (VI) complexes and being of sufficient concentration to prevent precipitation of ferrous, nickel, and molybdenum ions.

3. An aqueous electrolytic bath for use in the process of deposition of a ferromagnetic coating on an electrically conductive carrier in which process said carrier is subjected as a cathode to electrolytic action in said bath, said bath containing ferrous chloride, nickel chloride, and sodium molybdate and including as essential constituents ferrous ions in a concentration approximately 14 grams per liter, nickel ions in a concentration approximately 5 grams per liter, molybdate ions in a concentration approximately .7 gram per liter, and a complexing agent capable of forming soluble ferrous, nickel, and molybdate complexes and being of sufficient concentration to prevent precipitation of said ferrous, nickel, and molybdate ions, said bath having a pH of approximately 8.5.

4. An aqueous electrolytic bath for use in the process of deposition of a ferromagnetic coating on an electrically conductive carrier in which process said carrier is subjected as a cathode to electrolytic action in said bath, said bath containing ferrous chloride, nickel chloride, and sodium molybdate and including as essential constituents ferrous ions in a concentration approximately 14 grams per liter, nickel ions in a concentration approximately 5 grams per liter, molybdate ions in a concentration approximately .7 gram per liter, and a complexing agent consisting of citrate ions in a concentration approximately 104 grams per liter, said bath having a pH of approximately 8.5.

5. An aqueous electrolytic bath for use in the process of deposition of a ferromagnetic coating on an electrically conductive carrier in which process said carrier is subjected as a cathode to electrolytic action in said bath, said bath containing ferrous chloride, nickel chloride, and sodium molybdate and including as essential constituents ferrous ions in a concentration approximately 14 grams per liter, nickel ions in a concentration approximately 5 grams per liter, molybdate ions in a concentration approximately .7 gram per liter, ammonium ions in a concentration approximately 17 grams per liter, and a complexing agent consisting of citrate ions in a concentration approximately 42 grams per liter, said bath having a pH of approximately 8.5 by the addition of ammonium hydroxide.

concentration approximately 17 grams per liter, and a complexing agent consisting of citrate ions in a concentration approximately 104 grams per liter, said bath having a pH of approximately 8.5 by the addition of ammonium hydroxide.

6. An aqueous electrolytic bath for use in the process of deposition of a ferromagnetic coating on an electrically conductive carrier in which process said carrier is subjected as a cathode to electrolytic action in said bath, said bath having a pH in the range of 7.5 to 9.5 and including as essential constituents ferric ions in a concentration in the range of .7 to 3 grams per liter, nickel ions in a concentration in the range of 3 to 10 grams per liter, molybdenum (VI) in a concentration in the range of .1 to 1 gram per liter and a complexing agent capable of forming soluble ferric, nickel, and molybdenum (VI) complexes and being of sufficient concentration to prevent precipitation of ferric, nickel, and molybdenum (VI) ions.

7. An aqueous electrolytic bath for use in the process of deposition of a ferromagnetic coating on an electrically conductive carrier in which process said carrier is subjected as a cathode to electrolytic action in said bath, said bath having a pH of approximately 8.5 and including as essential constituents ferric ions in a concentration approximately 1 gram per liter, nickel ions in a concentration approximately 5 grams per liter, molybdenum (VI) in a concentration approximately .4 gram per liter, and a complexing agent capable of forming soluble ferric, nickel, and molybdenum (VI) complexes and being of sufficient concentration to prevent precipitation of ferric, nickel, and molybdenum ions.

8. An aqueous electrolytic bath for use in the process of deposition of a ferromagnetic coating on an electrically conductive carrier in which process said carrier is subjected as a cathode to electrolytic action in said bath, said bath containing ferric chloride, nickel chloride, and sodium molybdate and including as essential constituents ferric ions in a concentration approximately 1 gram per liter, nickel ions in a concentration approximately 5 grams per liter, molybdate ions in a concentration approximately .7 gram per liter, and a complexing agent capable of forming soluble ferric, nickel, and molybdate complexes and being of sufficient concentration to prevent precipitation of said ferric, nickel, and molybdate ions, said bath having a pH of approximately 8.5.

9. An aqueous electrolytic bath for use in the process of deposition of a ferromagnetic coating on an electrically conductive carrier in which process said carrier is subjected as a cathode to electrolytic action in said bath, said bath containing ferric chloride, nickel chloride, and sodium molybdate and including as essential constituents ferric ions in a concentration approximately 1 gram per liter, nickel ions in a concentration approximately 5 grams per liter, molybdate ions in a concentration approximately .7 gram per liter, and a complexing agent consisting of citrate ions in a concentration approximately 42 grams per liter, said bath having a pH of approximately 8.5.

10. An aqueous electrolytic bath for use in the process of deposition of a ferromagnetic coating on an electrically conductive carrier in which process said carrier is subjected as a cathode to electrolytic action in said bath, said bath containing ferric chloride, nickel chloride, and sodium molybdate and including as essential constituents ferric ions in a concentration approximately 1 gram per liter, nickel ions in a concentration approximately 5 grams per liter, molybdate ions in a concentration approximately .7 gram per liter, ammonium ions in a concentration approximately 17 grams per liter, and a complexing agent consisting of citrate ions in a concentration approximately 42 grams per liter, said bath having a pH of approximately 8.5 by the addition of ammonium hydroxide.

11. A process for fabricating magnetic computing de-

vices comprising the steps of: providing an aqueous electrolytic bath having a pH in the range of 7.5 to 9.5 and including as essential constituents iron ions in a concentration in the range of .7 to 16 grams per liter, nickel ions in a concentration in the range of 3 to 10 grams per liter, molybdenum (VI) in a concentration in the range of .1 to 1 gram per liter, and a complexing agent capable of forming soluble iron, nickel, and molybdenum complexes and being of sufficient concentration to prevent precipitation of iron, nickel, and molybdenum ions; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

12. A process for fabricating magnetic computing devices comprising the steps of: providing an aqueous electrolytic bath having a pH in the range of 7.5 to 9.5 and including as essential constituents ferrous ions in a concentration in the range of 12 to 16 grams per liter, nickel ions in a concentration in the range of 3 to 10 grams per liter, molybdenum (VI) in a concentration in the range of .1 to 1 gram per liter, and a complexing agent capable of forming soluble ferrous, nickel, and molybdenum (VI) complexes and being of sufficient concentration to prevent precipitation of ferrous, nickel, and molybdenum (VI) ions; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

13. A process for fabricating magnetic computing devices comprising the steps of: providing an aqueous electrolytic bath having a pH in the range of 7.5 to 9.5 and including as essential constituents ferrous ions in a concentration in the range of 12 to 16 grams per liter, nickel ions in a concentration in the range of 3 to 10 grams per liter, molybdenum (VI) in a concentration in the range of .1 to 1 gram per liter, and a complexing agent consisting of citrate ions in a concentration of 88 to 113 grams per liter; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

14. A process for fabricating magnetic computing devices comprising the steps of: providing an aqueous electrolytic bath having a pH in the range of 7.5 to 9.5 and including as essential constituents ferrous ions in a concentration in the range of 12 to 16 grams per liter, nickel ions in a concentration in the range of 3 to 10 grams per liter, molybdenum (VI) in a concentration in the range of .1 to 1 gram per liter, ammonium ions in a concentration in the range of 12 to 34 grams per liter, and a complexing agent capable of forming soluble ferrous, nickel, and molybdenum (VI) complexes and being of sufficient concentration to prevent precipitation of ferrous, nickel, and molybdenum (VI) ions; subject-

ing an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

15. A process for fabricating magnetic computing devices comprising the steps of: providing an aqueous electrolytic bath containing ferrous chloride, nickel chloride, and sodium molybdate and including as essential constituents ferrous ions in a concentration in the range of 12 to 16 grams per liter, nickel ions in a concentration in the range of 3 to 10 grams per liter, molybdate ions in a concentration in the range of .3 to 2 grams per liter, and a complexing agent, said bath having a pH in the range of 7.5 to 9.5; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

16. A process for fabricating magnetic computing devices comprising the steps of: providing an aqueous electrolytic bath containing ferrous chloride, nickel chloride, and sodium molybdate and including as essential constituents ferrous ions in a concentration in the range of 12 to 16 grams per liter, nickel ions in a concentration in the range of 3 to 10 grams per liter, molybdate ions in a concentration in the range of .3 to 2 grams per liter, and a complexing agent consisting of citrate ions in a concentration in the range of 88 to 113 grams per liter, said bath having a pH in the range of 7.5 to 9.5; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

17. A process for fabricating magnetic computing devices comprising the steps of: providing an aqueous electrolytic bath including as essential constituents ferrous ions in a concentration in the range of 12 to 16 grams per liter, nickel ions in a concentration in the range of 3 to 10 grams per liter, molybdenum (VI) in a concentration in the range of .1 to 1 gram per liter, ammonium ions in a concentration in the range of 12 to 34 grams per liter, and a complexing agent consisting of citrate ions in a concentration in the range of 88 to 113 grams per liter, said bath having a pH in the range of 7.5 to 9.5; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

18. A process for fabricating magnetic computing devices comprising the steps of: providing an aqueous electrolytic bath containing ferrous chloride, nickel chloride,

and sodium molybdate and including as essential constituents ferrous ions in a concentration in the range of 12 to 16 grams per liter, nickel ions in a concentration in the range of 3 to 10 grams per liter, molybdate ions in a concentration in the range of .3 to 2 grams per liter, ammonium ions in a concentration in the range of 12 to 34 grams per liter, and a complexing agent consisting of citrate ions in a concentration in the range of 88 to 113 grams per liter, said bath having a pH in the range of 7.5 to 9.5 by the addition of ammonium hydroxide; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

19. A process for fabricating magnetic computing devices comprising the steps of: providing an aqueous electrolytic bath having a pH in the range of 7.5 to 9.5 and including as essential constituents ferric ions in a concentration in the range of .7 to 3 grams per liter, nickel ions in a concentration in the range of 3 to 10 grams per liter, molybdenum (VI) in a concentration in the range of .1 to 1 gram per liter, and a complexing agent capable of forming soluble ferric, nickel, and molybdenum (VI) complexes and being of sufficient concentration to prevent precipitation of ferric, nickel, and molybdenum (VI) ions; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

20. A process for fabricating magnetic computing devices comprising the steps of: providing an aqueous electrolytic bath having a pH in the range of 7.5 to 9.5 and including as essential constituents ferric ions in a concentration in the range of .7 to 3 grams per liter, nickel ions in a concentration in the range of 3 to 10 grams per liter, molybdenum (VI) in a concentration in the range of .1 to 1 gram per liter, and a complexing agent consisting of citrate ions in a concentration of 33 to 104 grams per liter; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

21. A process for fabricating magnetic computing devices comprising the steps of: providing an aqueous electrolytic bath having a pH in the range of 7.5 to 9.5 and including as essential constituents ferric ions in a concentration in the range of .7 to 3 grams per liter, nickel ions in a concentration in the range of 3 to 10 grams per liter, molybdenum (VI) in a concentration in the range of .1 to 1 gram per liter, ammonium ions in a concentration in the range of 8 to 25 grams per liter, and a complexing agent capable of forming soluble ferric, nickel, and molybdenum (VI) complexes and being of sufficient concentration to prevent precipitation of ferric, nickel, and molybdenum (VI) ions; subjecting

an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

22. A process for fabricating magnetic computing devices comprising the steps of: providing an aqueous electrolytic bath containing ferric chloride, nickel chloride, and sodium molybdate and including as essential constituents ferric ions in a concentration in the range of .7 to 3 grams per liter, nickel ions in a concentration in the range of 3 to 10 grams per liter, molybdate ions in a concentration in the range of .3 to 2 grams per liter, and a complexing agent capable of forming soluble ferric, nickel, and molybdate complexes and being of sufficient concentration to prevent precipitation of said ferric, nickel, and molybdate ions, said bath having a pH in the range of 7.5 to 9.5; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

23. A process for fabricating magnetic computing devices comprising the steps of: providing an aqueous electrolytic bath containing ferric chloride, nickel chloride, and sodium molybdate and including as essential constituents ferric ions in a concentration in the range of .7 to 3 grams per liter, nickel ions in a concentration in the range of 3 to 10 grams per liter, molybdate ions in a concentration in the range of .3 to 2 grams per liter, and a complexing agent consisting of citrate ions in a concentration in the range of 33 to 104 grams per liter, said bath having a pH in the range of 7.5 to 9.5; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

24. A process for fabricating magnetic computing devices comprising the steps of: providing an aqueous electrolytic bath including as essential constituents ferric ions in a concentration in the range of .7 to 3 grams per liter, nickel ions in a concentration in the range of 3 to 10 grams per liter, molybdenum (VI) in a concentration in the range of .1 to 1 gram per liter, ammonium ions in a concentration in the range of 8 to 25 grams per liter, and a complexing agent consisting of citrate ions in a concentration in the range of 33 to 104 grams per liter, said bath having a pH in the range of 7.5 to 9.5; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said carrier, by an amount sufficient to establish in said coating an easy direction of magnetization which is oriented at an angle with respect to said longitudinal axis.

25. A process for fabricating magnetic computing devices comprising the steps of: providing an aqueous electrolytic bath containing ferric chloride, nickel chloride, and sodium molybdate and including as essential constituents ferric ions in a concentration in the range of .7 to 3 grams per liter, nickel ions in a concentration in the range of 3 to 10 grams per liter, molybdate ions in a concentration in the range of .3 to 2 grams per liter, ammonium ions in a concentration in the range of 8 to 25 grams per liter, and a complexing agent consisting of citrate ions in a concentration in the range of 33 to 104 grams per liter, said bath having a pH in the range of 7.5 to 9.5 by the addition of ammonium hydroxide; subjecting an elongated electrically conductive carrier as a cathode to electrolytic action in said bath for a time sufficient to effect the deposition thereon of a ferromagnetic coating which has the property of providing a particularly oriented easy direction of magnetization when stressed; and applying a torsional stress to said coating, relative to a longitudinal axis of said car-

rier, by an amount sufficient to establish in said coating an easy direction of magnetization which is oriented at an angle with respect to said longitudinal axis.

## References Cited in the file of this patent

## UNITED STATES PATENTS

|           |                    |               |
|-----------|--------------------|---------------|
| 1,837,355 | Burns et al. ----- | Dec. 22, 1931 |
| 2,507,400 | Marinis -----      | May 9, 1950   |
| 2,599,178 | Holt et al. -----  | June 3, 1952  |

## FOREIGN PATENTS

|        |                 |               |
|--------|-----------------|---------------|
| 18,378 | Australia ----- | Oct. 22, 1929 |
|--------|-----------------|---------------|

## OTHER REFERENCES

15 Ernst et al.: Jour. Electrochemical Soc., vol. 102 (August 1955), pp. 461-469.  
 Haymes: Elements of Magnetic Tape Recording, 1957, p. 38.  
 20 Bobeck: "Bell System Technical Journal," November 1957, vol. XXXVI, pp. 1319-1340.